

## 1

3,266,994

PROCESS AND COMPOSITION FOR  
TREATING OF HAIR

Carroll R. Reiss, Green Township, Hamilton County, and  
J. Leon Lichtin, Springfield Township, Hamilton County,  
Ohio, assignors to The Realistic Company, Cincinnati,  
Ohio, a corporation of Ohio  
No Drawing. Filed June 24, 1963, Ser. No. 290,183  
9 Claims. (Cl. 167—87.1)

This invention relates to the treatment of hair as in the permanent waving thereof.

An object of this invention is to provide an improved process for waving the hair and chemicals for use in waving the hair.

A further object of this invention is to provide a hair waving method and chemicals for use in hair waving which produce curls which retain a tight uniform helical shape on drying and which maintains its improved shape after repeated washings or other treatments which normally weaken curl structure.

In the waving of hair, it is common practice to soften or treat the hair with a reducing solution such as a solution of thioglycolic acid and ammonium hydroxide in water which produces changes in the hair by reducing keratin and which softens the hair to permit shaping of the hair on a mandrel such as a curling rod or the like. An oxidizing agent is applied to the treated hair to neutralize that portion of the reducing agent which remains on the hair and to oxidize the reduced keratin to restore the strength thereof, but the strength is only partially restored upon treatment with the oxidizing agent. According to our improved method, we add a water-soluble, non-toxic salt of a polyvalent metal such as magnesium sulfate, aluminum sulfate, calcium acetate, calcium chloride, or the like to an aqueous solution of reducing agent. Alternatively, we employ an aqueous solution of an oxidizing salt of a polyvalent metal such as magnesium bromate, calcium bromate, aluminum bromate or the corresponding iodates or mixtures thereof in neutralizing and treating reduced keratin of the hair. The hair fibres of waves neutralized with our improved compositions have a substantially greater tensile strength than hair fibres neutralized with conventional oxidizing solutions, and the waves are longer lasting and have a lesser tendency for fibres to separate from one another.

Oxidizing agents with which our salts can be used include water-soluble ammonium, alkali and alkaline earth bromates, iodates, and periodates, hydrogen peroxide, and urea peroxide and the like.

Mixtures of the oxidizing agent and polyvalent salt can be made to form a mixture which can be dissolved in water, and in such a mixture, the oxidizing agent and polyvalent salt can be mixed in approximately the ratio desired in the neutralizing solution. An example of such a mixture contains 100 parts of sodium bromate and 280 parts of  $MgSO_4 \cdot 7H_2O$ , all parts being by weight. In the neutralizer solution, it is preferred to have substantially as great a concentration of polyvalent salt as can be maintained in solution conveniently in order to obtain the maximum effect from the polyvalent salt, but lesser concentrations can be used if desired.

## 2

The following examples are given to illustrate the invention in greater detail, but it is to be understood that the examples are given primarily by way of example, rather than by way of limitation, except as set forth in the claims. In the following examples and in the remainder hereof, all parts or percentages are given by weight.

## Example I

A tress of hair including approximately 12 fibres of human hair was wrapped around a quarter-inch mandrel in helical fashion, for three complete revolutions and held in place thereon. The tress was immersed in a reductant solution containing 7.0% thioglycolic acid and sufficient ammonia to provide an excess and give a pH of 9.4. The tress was immersed in the reductant for approximately 7 minutes and was then rinsed thoroughly in tepid water. The tress was then immersed in a neutralizer solution which contained 100 parts of sodium bromate, 280 parts of  $MgSO_4 \cdot 7H_2O$ , 3 parts of sodium lauryl ether sulfate together with sufficient sulfuric acid to bring the composition to a pH of 6.0 and sufficient water to make 1,000 parts of neutralizer solution. The tress was immersed in the neutralizer for 7 minutes. The tress was then rinsed in tepid water and removed from the mandrel. On drying in air, the tress retained its uniform helical shape with very little change in diameter and the individual fibres showed no tendency to lose their helical shape or separate from one another. On immersion in water, the tress exhibited practically no motion at all, neither expanding into a large helix nor contracting into a tight knotted configuration.

## Example II

A tress of hair including approximately 12 fibres of human hair was wrapped around a quarter-inch mandrel in helical fashion, for three complete revolutions and held in place thereon. The tress was immersed in a reductant solution containing 7.0% thioglycolic acid and sufficient ammonia to provide an excess and give a pH of 9.4. The tress was immersed in the reductant for approximately 7 minutes and was then rinsed thoroughly in tepid water. The tress was then immersed in a neutralizer solution which contained 100 parts of sodium bromate, 180 parts of  $Ca(C_2H_3O_2)_2 \cdot H_2O$ , 3 parts of sodium lauryl ether sulfate, sufficient sulfuric acid to bring the composition to a pH of 6.0 and sufficient water to make 1,000 parts of neutralizer. The tress was immersed in the neutralizer for 7 minutes. The tress was then rinsed in tepid water and removed from the mandrel. On drying in air, the tress retained its uniform helical shape with very little change in diameter and the individual fibres showed no tendency to lose their helical shape or separate from one another.

## Example III

A tress of hair including approximately 12 fibres of human hair was wrapped around a quarter-inch mandrel in helical fashion, for three complete revolutions and held in place thereon. The tress was immersed in a reductant solution containing 7.0% thioglycolic acid and sufficient ammonia to provide an excess and give a pH of 9.4. The tress was immersed in the reductant for approximately 7 minutes and was then rinsed thoroughly in tepid water.

The tress was then immersed in a neutralizer solution. In the preparation of the neutralizer, 100 parts of sodium bromate, 15 parts of boric acid and 3 parts of sodium alkyl phenoxyether sulfonate were dissolved in 882 parts of water to form a first solution. 38 parts of



were dissolved in 62 parts of the first solution, and the resultant neutralizer solution was used at once. The tress was immersed in the neutralizer solution for 7 minutes. The tress was then rinsed in tepid water and removed from the mandrel. On drying in air, the tress retained its uniform helical shape with very little change in diameter and the individual fibres showed no tendency to lose their helical shape or separate from one another.

*Example IV*

A tress of hair including approximately 12 fibres of human hair was wrapped around a quarter-inch mandrel in helical fashion, for three complete revolutions and held in place thereon. The tress was immersed in a reductant solution containing 7.0% thioglycolic acid and sufficient ammonia to provide an excess and give a pH of 9.4. The tress was immersed in the reductant for approximately 7 minutes and was then rinsed thoroughly in tepid water. The tress was then immersed in a neutralizer solution which contained 20 parts of sodium periodate, 200 parts of  $\text{MgSO}_4 \cdot 7\text{H}_2\text{O}$  and sufficient water to make 1,000 parts of neutralizer. The tress was immersed in the neutralizer for 7 minutes. The tress was then rinsed in tepid water and removed from the mandrel. On drying in air, the tress retained its uniform helical shape with very little change in diameter and the individual fibres showed no tendency to lose their helical shape or separate from one another.

*Example V*

A tress of hair including approximately 12 fibres of human hair was wrapped around a quarter-inch mandrel in helical fashion, for three complete revolutions and held in place thereon. The tress was immersed in a reductant solution containing 7.0% thioglycolic acid and sufficient ammonia to provide an excess and give a pH of 9.4. The tress was immersed in the reductant for approximately 7 minutes and was then rinsed thoroughly in tepid water. The tress was then immersed in a neutralizer solution which contained 20 parts of sodium periodate, 300 parts of  $\text{MgSO}_4 \cdot 7\text{H}_2\text{O}$  and sufficient water to make 1,000 parts of neutralizer. The tress was immersed in the neutralizer for 7 minutes. The tress was then rinsed in tepid water and removed from the mandrel. On drying in air, the tress retained its uniform helical shape with very little change in diameter and the individual fibres showed no tendency to lose their helical shape or separate from one another.

*Example VI*

A tress of hair including approximately 12 fibres of human hair was wrapped around a quarter-inch mandrel in helical fashion, for three complete revolutions and held in place thereon. The tress was immersed in a reductant solution containing 7.0% thioglycolic acid and sufficient ammonia to provide an excess and give a pH of 9.4. The tress was immersed in the reductant for approximately 7 minutes and was then rinsed thoroughly in tepid water. The tress was then immersed in a neutralizer solution which contained 250 parts of commercial 6% hydrogen peroxide solution in water, 200 parts of



and sufficient water to make 1,000 parts of neutralizer. The tress was immersed in the neutralizer for 7 minutes. The tress was then rinsed in tepid water and removed from the mandrel. On drying in air, the tress retained its uniform helical shape with very little change in diameter

and the individual fibres showed no tendency to lose their helical shape or separate from one another.

The neutralizing composition and method of treating hair are subject to variation within the spirit and scope of the appended claims.

Having described our invention, what we claim as new and desire to protect by Letters Patent is:

1. In a process for treating hair to impart a permanent set thereto which includes the steps of treating the hair with a reducing agent for keratin and then treating the hair with an aqueous solution of an oxidizing agent for reduced keratin, the improvement which comprises including in the solution of oxidizing agent at least 18 percent by weight of a water soluble non-toxic salt of a polyvalent metal selected from the group consisting of magnesium, aluminum, and calcium.

2. In a process for treating hair to impart a permanent set thereto which includes the steps of treating the hair with a reducing agent for keratin and then treating the hair with an aqueous solution of an oxidizing agent for reduced keratin, the improvement which comprises including in the solution of oxidizing agent at least 20 percent by weight of magnesium sulfate.

3. In a process for treating hair to impart a permanent set thereto which includes the steps of treating the hair with a reducing agent for keratin and then treating the hair with an aqueous solution of an oxidizing agent for reduced keratin, the improvement which comprises including in the solution of oxidizing agent at least 38 percent by weight of aluminum sulfate.

4. In a process for treating hair to impart a permanent set thereto which includes the steps of treating the hair with a reducing agent for keratin and then treating the hair with an aqueous solution of an oxidizing agent for reduced keratin, the improvement which comprises including in the solution of oxidizing agent approximately 18 to 20 percent by weight of calcium acetate.

5. In a process for treating hair to impart a permanent set thereto which includes the steps of treating the hair with a reducing agent for keratin and then treating the hair with an aqueous solution of an oxidizing agent selected from the group consisting of soluble ammonium, alkali, and alkaline earth iodates, periodates, and bromates, hydrogen peroxide and urea peroxide, the improvement which comprises including in the solution of oxidizing agent at least 18 percent by weight of a water-soluble non-toxic salt of a polyvalent metal selected from the group consisting of magnesium, calcium and aluminum.

6. In a process for treating hair to impart a permanent set thereto which includes the steps of treating the hair with a reducing agent for keratin and then treating the hair with an aqueous solution of an oxidizing agent selected from the group consisting of soluble ammonium, alkali, and alkaline earth iodates, periodates, and bromates, hydrogen peroxide and urea peroxide, the improvement which comprises including in the solution of oxidizing agent 20 to 30 percent by weight of magnesium sulfate.

7. In a process for treating hair to impart a permanent set thereto which includes the steps of treating the hair with a reducing agent for keratin and then treating the hair with an aqueous solution of an oxidizing agent selected from the group consisting of soluble ammonium, alkali, and alkaline earth iodates, periodates, and bromates, hydrogen peroxide and urea peroxide, the improvement which comprises including in the solution of oxidizing agent approximately 38 percent by weight of aluminum sulfate.

8. In a process for treating hair to impart a permanent set thereto which includes the steps of treating the hair with a reducing agent for keratin and then treating the hair with an aqueous solution of an oxidizing agent selected from the group consisting of soluble ammonium, alkali, and alkaline earth iodates, periodates, and bromates, hydrogen peroxide and urea peroxide, the improvement

which comprises including in the solution of oxidizing agent approximately 18 to 20 percent by weight of calcium acetate.

9. A hair treating composition which consists essentially of an aqueous solution of sodium bromate and at least 20 percent by weight of magnesium sulfate.

References Cited by the Examiner

FOREIGN PATENTS

992,156 10/1951 France.  
295,538 3/1954 Switzerland.

OTHER REFERENCES

De Navarre: American Perfumer and Essential Oil Review, January 1950, page 21.

5 Sargarin: Cosmetics: Sience and Technology, published by Interscience Publishers, Inc., N.Y., 1957, pp. 609, 619 and 620.

LEWIS GOTTS, *Primary Examiner.*

10 FRANK CACCIAPAGLIA, JR., *Examiner.*

RICHARD L. HUFF, *Assistant Examiner.*